

## UNITED STATES PATENT OFFICE

2,408,103

## MINERAL OIL COMPOSITION

Herschel G. Smith, Wallingford, and Troy L. Cantrell, Lansdowne, Pa., and John G. Peters, Audubon, N. J., assignors to Gulf Oil Corporation, Pittsburgh, Pa., a corporation of Pennsylvania

No Drawing. Application March 19, 1945.  
Serial No. 583,659

5 Claims. (Cl. 252—39)

1

This invention relates to improved mineral oil compositions, and more particularly to improved mineral oils and oil compositions each comprising a major amount of mineral oil and a minor amount of a new improvement agent, or mixture of agents, capable of imparting a plurality of useful, advantageous properties thereto; these improved oil compositions being useful and advantageous in protecting metals, both ferrous and non-ferrous metals, from rust, corrosion and wear. It also includes methods of making such agents and improved oil compositions containing the same.

As is well known, the simple straight mineral oils usually are deficient in one or more respects, for certain commercial uses and it is common practice to incorporate one or more "additive" compounds in the oil to overcome the defect or defects thereof for certain uses. Likewise, various agents have been incorporated in oils to improve certain of their properties for particular or special uses requiring a superior oil. In general, such agents or additive compounds are known as improvement agents.

We have now discovered certain new improvement agents for mineral oils which are particularly advantageous in the commercial preparation of various lubricants, protective coating compositions and other useful mineral oil compositions. Our agents can be readily incorporated in various mineral oils and oil compositions. When incorporated therein, even in very small amounts, these agents markedly improve the rust preventive qualities thereof. Further, they are also capable of imparting other useful and advantageous properties to mineral oil and oil compositions, as more fully described post.

Our new and advantageous improvement agents for mineral oils and oil compositions are oil-soluble metal salts having the following formula:



wherein M is a divalent metal, such as calcium, etc., R is an alkyl group containing from 8 to 22 carbon atoms and R' is hydrogen or an alkyl group, advantageously a short chain alkyl group. That is, our improvement agents are substan-

2

tially neutral divalent metal salts of ortho phthalimic acids containing two alkyl groups attached to the nitrogen atom thereof, one being a hydroxylated alkyl group and the other a long chain alkyl group, as shown by the above formula.

As a class, the above metal salts are excellent improvement agents for mineral oils and oil compositions and can be easily incorporated in such oil compositions, in proportions necessary for present purposes. All of these improvement agents are readily and markedly soluble in mineral oils, particularly naphthenic type oils. Indeed, most of them are viscous oily liquids at ordinary temperatures and can be readily incorporated in paraffinic type mineral oils, as well as naphthenic and mixed type base oils. Again, some of them are waxy solids or oily semi-solids at ordinary room temperature, i. e. 75° F., but soften or melt at elevated temperatures; they being viscous liquids at elevated temperatures below their decomposition point. Thus, in general, our improvement agents can be readily fluxed or blended with a wide variety of mineral oils and oil compositions and when incorporated therein improve various properties thereof.

On the other hand, our new improvement agents are water-resistant compounds which are practically insoluble in water and aqueous solutions. That is, they have a combination of properties which render them particularly advantageous for the purposes of this invention, as is shown more fully post.

Further, these improvement agents can be readily prepared by various methods, as described in our companion application Serial No. 608,100, filed July 31, 1945, wherein we claim these new oil-soluble metal salts and methods of making the same. As there described, our new improvement agents can be readily prepared, advantageously in situ in mineral oil, directly from divalent metal hydroxides, phthalic anhydride and secondary aliphatic amines having the following formula:



wherein R' represents hydrogen or an alkyl group and R represents an alkyl group containing from 8 to 22 carbon atoms. In turn, these secondary alkyl amines containing a hydroxyl group attached to one of the alkyl groups thereof can be readily prepared by reacting alkylene oxides such as ethylene oxide, propylene oxide, butylene oxide

3 and the like with primary alkyl amines having the following formula:



5 wherein  $n$  is a number between 6 and 18. Some of the primary alkyl amines of this generic class are

Mono-capryl amine  
Mono-lauryl amine  
Mono-myristyl amine  
Mono-palmityl amine  
Mono-stearyl amine

15 and other primary alkyl amines having the above formula. Any of the above primary fatty amines may be used with advantage in making the secondary amines useful for the present purposes, as all of them readily react with propylene oxide and similar alkylene oxides, as shown in our said, companion application, Serial No. 608,100. For instance, as there shown, mono-lauryl amine (primary dodecyl amine) is useful and advantageous. Likewise, primary hexadecyl amine (mono-palmityl amine) is also advantageous in preparing secondary aliphatic amines useful for the present purposes. Further, mixtures of such primary amines may also be employed, somewhat better products being obtained with mixed amines. For instance, one commercially available mixture of such primary fatty amines is the so-called "cocoamine". As stated in the said copending application, commercial "cocoamine" has an average molecular weight of 210 and contains a major amount of lauryl amine admixed with minor amounts of homologues thereof. This commercial fatty amine may be employed with advantage in preparing secondary aliphatic amines useful in making our improved oil-soluble polyvalent metal salts of ortho phthalamic acids by the advantageous methods set forth in our copending application Serial No. 608,100.

Further, as shown in our said copending application, in so preparing our agents from such secondary amines, phthalic anhydride and divalent metal hydroxide, those chemicals are reacted together and converted into new compounds; they being chemically combined together in the molecular ratios necessary to produce our new substantially neutral oil-soluble divalent metal salts having substantially the generic structure given ante. In doing so, we usually react said secondary amines with phthalic anhydride in substantially equimolecular amounts to form a monoamide of phthalic acid, namely, the desired N-alkyl, N-alkyloxy ortho phthalamic acid, and then neutralize the residual acidity of that compound by reaction with lime, sufficient lime being employed to form substantially neutral lime salts thereof. In lieu of lime, other hydroxides of divalent metals may be employed such as magnesium hydroxide, barium hydroxide and the like. Further, in so preparing these metal salts, these reactions can be advantageously effected in the presence of sufficient mineral oil to dissolve the oil-soluble compound so obtained; the new improvement agents being formed in situ in the oil, as described and illustrated in our said companion application Serial No. 608,100.

Indeed, in the practice of the present invention we usually prepare the desired metal salts in situ in mineral oil. The concentrated solutions of neutral metal salts in oil have certain advantages for the present purposes; they being

themselves excellent improvement agents for imparting rust preventive qualities and other advantageous properties to a wide range of commercial compositions, such as greases, waxes, petrolatum and petrolatum-like coating compositions, as well as mineral oils and oil compositions.

10 The following examples illustrate various methods of preparing our improvement agents and improved compositions containing the same.

Example I.—In this example, a substantially neutral calcium salt was prepared, in situ in mineral oil, directly from phthalic anhydride, dodecyl propanol amine and hydrated lime; the oil-soluble salt so prepared being a neutral calcium salt of N-dodecyl, propanol ortho phthalamic acid and having the following formula:



30 The procedure in preparing this improvement agent was as follows: To 1640 grams of a 70 viscosity Texas oil distillate were added 296 grams of phthalic anhydride and 74 grams of hydrated lime. The lime, phthalic anhydride, oil slurry was then stirred vigorously while 486 grams of dodecyl propanol amine were added over the course of one hour. During this time the temperature was maintained at 150° F. and after the lime and phthalic anhydride had gone into solution, the temperature was raised to 280° F. and the oil solution was filtered.

35 The filtrate so obtained is an excellent improvement agent for present purposes. This oily mobile liquid agent had the following properties:

40 Gravity: A. P. I. 18.3  
Viscosity, S. U. V. 432  
100° F. 56.9  
45 210° 5.58  
Ash as sulfate

50 It was a concentrated solution of the said neutral calcium salt and contained approximately 33 per cent by weight of said calcium salt. Nevertheless, it was a light mobile liquid at room temperature. This clearly shows the high solubility of our new metal salts in mineral oils.

55 That is, the foregoing example is typical and illustrative of certain embodiments of this invention. In other embodiments thereof, other secondary alkyl, alkylol amines can also be employed in making our improvement agents as stated ante. For instance, in Example I, other secondary amines such as dodecyl butanol amine, 60 hexadecyl propanol amine and the like may be employed in lieu of dodecyl propanol amine. Further, mixtures of such secondary alkyl, alkylol amines may likewise be employed with advantage, as illustrated in the following examples:

65 Example II.—This example illustrates the preparation of a mixture of secondary amines which are useful in making our oil-soluble metal salts; this mixture of secondary alkyl alkylol amines being typical and advantageous for the present purposes and being prepared from propylene oxide and commercial cocoamine.

70 Into a suitable reaction vessel equipped with a reflux condenser and means for heating and agitating the charge, there were charged 840 grams of commercial cocoamine and then 232

grams of propylene oxide were gradually added to the amine with stirring. After the reactants were intimately admixed the mixture was allowed to stand over night. Then the reaction mixture was refluxed for five hours on a water bath to complete the reaction.

The reaction product so obtained was a homogeneous, clear, semi-viscous liquid comprising a mixture of secondary fatty propanol amines containing a major amount of lauryl propanol amine. This mixture of secondary amines is useful and advantageous in preparing a wide variety of our new oil-soluble improvement agents. It readily reacts with phthalic anhydride to form ortho phthalamic acid which in turn can be readily converted into various metal salts by reaction with divalent metal hydroxides.

The preparation of one advantageous improvement agent from this mixture of secondary fatty propanol amines is illustrated in the following example.

*Example III.*—In this example, a substantially neutral calcium salt was prepared, *in situ* in a light mineral lubricating oil, directly from phthalic anhydride, hydrated lime and the mixture of secondary amines obtained in Example II ante; the mineral oil being a 70 viscosity Texas oil distillate having the following properties:

|                      |         |
|----------------------|---------|
| Gravity: °A. P. I.   | 26.0    |
| Viscosity, S. U. V.: |         |
| 100° F.              | sec. 70 |
| 210°                 | 36      |

In preparing this advantageous improvement agent, the following procedure was employed.

To 1780 grams of the mineral oil were added 296 grams of phthalic anhydride and 74 grams of hydrated lime. The lime, phthalic anhydride oil slurry was then stirred vigorously while 536 grams of the secondary amines were added over the course of one hour. During this time the temperature was maintained at 150° F. and after the lime and phthalic anhydride had gone into solution, the temperature was raised to 280° F. and the oil solution was filtered.

The filtrate so obtained is also an excellent improvement agent for the present purposes. It was an oily mobile liquid at room temperature and had the following properties:

|                    |      |
|--------------------|------|
| Gravity: °A. P. I. | 18.3 |
| Viscosity, SUV:    |      |
| 100° F.            | 432  |
| 210°               | 56.9 |

Ash as sulfate 5.1

It was a concentrated solution of substantially neutral calcium salts of the ortho phthalamic acids derived from said secondary amines. This oil solution contained approximately 33 per cent by weight of said calcium salts. Nevertheless, it was a light mobile liquid at room temperature. This clearly shows the high solubility of such salts in mineral oils.

This improvement agent had a good color and was substantially free of insoluble matter. It was readily miscible with various mineral oils and oil compositions and was directly soluble in most mineral oils in a manner effective for the present purposes. In particular, this improvement agent is useful and advantageous as an additive compound in preparing improved motor oils and like lubricants. It is also advantageous in preparing other improved oil compositions useful in protecting metals against abrasion and corrosion.

That is, the foregoing Examples I and III, respectively, are typical and illustrative of our new improvement agents and methods of making the same which are advantageous in certain embodiments of this invention. In other embodiments thereof, we may also employ various other divalent metal hydroxides and secondary amines containing an alkylol group in making our improvement agents, as stated ante. For instance, the hydroxides of magnesium, barium and other divalent metals may be used in Examples I and III, ante, in lieu of lime, to produce still other advantageous improvement agents.

In fact, by the present invention a wide range of improvement agents can be readily prepared in the generic practice thereof. All of them are readily soluble in commercial mineral oils and oil compositions in the proportions required to effect the desired improvements. Indeed, a wide range of improved anti-rust lubricants can be readily prepared by incorporating minor amounts of our improvement agents in suitable oils and oil compositions. In general, such improved anti-rust lubricants effectively protect ferrous and non-ferrous metals against rusting and corrosion, even when exposed to salt water and other severe conditions.

For instance, advantageous anti-rust lubricants can be prepared by dissolving in light lubricating oils small amounts of the products obtained in Examples I and III ante.

Further, the concentrated solutions of the calcium salts in oil, obtained in Examples I and III, are directly useful as rust preventive coating compositions for metals. They are substantially non-corrosive to both ferrous and non-ferrous metals. When applied to such metals, they tightly adhere to the metal forming a protective coating thereon which is resistant to water and aqueous liquids and fully protects the metal against rust or corrosion, even when exposed to the most drastic conditions. That is, our new oil-soluble metal salts are very potent rust preventive compounds. Accordingly, they can also be compounded with various other materials in preparing a wide range of protective coating compositions for metals. In particular, they are readily soluble in various hydrocarbon oils, particularly mineral lubricating oils. Further, they are also readily miscible with waxes, petrolatum and greases, as well as oil compositions.

Thus, our new improvement agents, such as obtained in Examples I and III, are useful in preparing a wide range of compositions having exceptional rust preventive properties; they being particularly advantageous in preparing improved anti-rust lubricants to which they impart further advantageous properties as shown post. Such improved lubricants can be readily obtained by incorporating small amounts of our improvement agents in mineral lubricating oils, greases, petrolatum and the like. For instance, the improvement agents obtained in Examples I and III are readily soluble in commercial mineral lubricating oils and when dissolved therein, even in small quantities markedly improve various properties of such oil. For example, the mineral lubricating oils containing from 0.1 to 1.0 per cent by weight of such improvement agents have increased resistance to oxidation and deterioration, as well as improved rust preventing or corrosion preventing properties.

The following examples illustrate the preparation of such improved lubricants and methods of making the same:

*Example IV.*—In this example one such advantageous anti-rust lubricant containing 0.1 per cent of the substantially neutral calcium salt of N-dodecyl propanol ortho phthalamic acid, dissolved in a commercial mineral lubricating oil was prepared as follows:

Into a suitable vessel, equipped with means for agitating the charge, there were charged 100 parts of the commercial lubricating oil and then 3 parts by weight of the filtrate obtained in Example I were added to the oil with stirring. The stirring was continued until the improved agent was uniformly and homogeneously blended with the oil.

The properties of the improved oil and the base oil employed in making the same were as follows:

|                     | Improved oil | Base oil |
|---------------------|--------------|----------|
| Gravity, ° A. P. I. | 30.0         | 30.0     |
| Viscosity, S.U.V.:  |              |          |
| 100° F.             | 102.8        | 102.8    |
| 210°                | 38.7         | 38.7     |
| Neutralization No.  | Nil          | Nil      |

As shown by the above tabulation of properties, the incorporation of this improvement agent in the base oil did not substantially change the physical properties thereof.

However, the improved oil so obtained had markedly improved rust-preventive qualities. For instance, when subjected to various standard corrosion tests, it completely inhibited rusting of the metal, whereas the base oil gave little or no protection against rust. In one such set of comparative tests the following data was obtained.

| Corrosion test, Method 412, Gulf                   | Improved oil | Base oil |
|----------------------------------------------------|--------------|----------|
| Distilled water, 122° F., 12 days—Steel strip:     |              |          |
| Appearance                                         | Bright       | Rusted   |
| Area rusted, per cent                              | 0            | 100      |
| Synthetic sea water, 122° F., 12 days—Steel strip: |              |          |
| Appearance                                         | Bright       | Rusted   |
| Area rusted, per cent                              | 0            | 100      |

The said corrosion tests employed were standard tests for determining the rust-preventive properties of commercial mineral oils and oil compositions. In such tests the procedure is as follows:

Thirty-six cc. of the oil to be tested and 4 cc. of distilled water are placed in a 1" x 6" Pyrex test tube, a polished steel strip is inserted in the oil-water mixture, and 2000 cc. of humid air per hour are bubbled through the mixture from a point near the bottom of the tube, so as to provide aeration and mixing of the oil and water; the apparatus being set in a water bath maintained at 122° F. (50° C.) and the original water level in the tube maintained by additions of fresh water every 24 hours. This test is continued for 12 days after which the test strip is removed and inspected.

A like test is also employed, for which straight sea water (or synthetic sea water) is used instead of distilled water. This variation is a far more severe corrosion test, the corrosion effects being usually ten or more times those for fresh water, other testing conditions being the same.

As shown by the test data ante, our improved anti-rust oil had outstanding rust-preventive properties and satisfactorily passed said test, particularly the drastic test with sea water.

In view of their outstanding anti-rust properties and other advantageous properties shown ante, our improvement agents are useful and advantageous in a wide range of commercial oil compositions. They may also be incorporated in minor amounts in other types of oils, such as turbine oils, instrument oils, electric motor oils and other high quality lubricants where it is important to protect metal surfaces from rust and corrosion, as well as adequate lubrication thereof under service conditions.

For example, improved turbine oils can be readily prepared by dissolving 0.03 to 3.0 per cent of our improvement agents, such as obtained in Examples I and III, in any of the commercial turbine oils. The preparation of one such improved turbine oil is illustrated in the following example:

*Example V.*—In this example, an improved turbine oil was prepared by dissolving 0.03 per cent of the filtrate obtained in Example III, in a suitable well-refined mineral lubricating oil. The improved lubricant contained 0.01 per cent of the substantially neutral calcium salts of the phthalamic acids obtained in said Example III.

The properties of this improved lubricant and the base oil employed in making the same were as follows:

|                     | Properties | Improved oil | Base oil |
|---------------------|------------|--------------|----------|
| Gravity, ° A. P. I. | 31.6       | 31.7         |          |
| Viscosity, S.U.V.:  |            |              |          |
| 100° F.             | 297        | 295          |          |
| 35 Flash, OC. ° F.  | 425        | 425          |          |
| Fire, OC. ° F.      | 470        | 470          |          |
| Pour, ° F.          | +5         | +5           |          |
| Color, N.P.A.       | 2.25       | 2.25         |          |
| Neutralization No.  | 0.02       | 0.02         |          |

40 The above improved turbine oil, with this markedly low dosage of our highly effective corrosion preventive agent, and without the addition of any supplemental corrosion preventive agent, successfully passed without any traces of rusting, 50 the above described steel strip corrosion test at a temperature of 122° F. for a test period of twelve days. Furthermore, it also passed the tentative test of the American Society for testing materials designated as ASTM D 665-42T, which is a similar test, but involves continuous mechanical stirring of a mixture of 90 per cent by volume of the oil and 10 per cent of distilled water at 140° F. for 48 hours. After the termination of this test there was no trace of corrosion for the standard steel 55 corrosion strip. Before the addition of the small amount of the anti-corrosion agent like tests by the two methods on the base oil both failed, with marked rusting, which began to appear in less than 12 hours from the start of each test.

60 In general, our improvement agents have proven to be quite satisfactory addition agents for turbine oils; particularly for compounded turbine oils of higher viscosity types, such as are preferred for marine service, the preferred 65 amount of the agent ranging from 0.01 per cent to 0.04 per cent according to our regular practice, although somewhat larger amounts of additive agent can be used without reducing the quality of the oil in other respects. For an actual 70 marine service test, an improved turbine oil testing 300 viscosity at 100° F. containing 0.01 per cent by weight of our improvement agent satisfactorily lubricated the turbines of an ocean going vessel under severe operating conditions. After 75 trial of 200 days, the lubricating system of the

turbine and auxiliary equipment were all free of rust or like corrosion. Further, the non-rusting quality of the improved turbine oil was found to be practically unchanged; a sample of the used oil, when tested for anti-rust and lubricating properties, was found to have retained its desired properties in all respects. The results from this run, along with others for similar operating conditions, demonstrate that the improved turbine oil is satisfactorily stable under service conditions and capable of operating satisfactorily for prolonged service in ocean going vessels; in particular, our improved turbine oils retain this important quality when exposed to oxidizing conditions or contact with water for long periods; that is, they retain this quality when exposed to oxidizing conditions of use, as well as the leaching effects of water for extended periods, due to the superior properties as regards resistance to oxidation and practical insolubility in water. Such improved turbine oils may be prepared as follows:

*Example VI.*—In this example, a superior improved turbine oil was prepared by admixing three parts of the filtrate obtained in Example III with 1000 parts of a commercial turbine oil containing incorporated therein 0.001 per cent of silicone polymer, as an antifoam agent. The mixture was agitated until a homogeneous blend was obtained.

The properties of said commercial turbine oil and the improved turbine oil prepared therefrom as above, were as follows:

|                                    | Improved oil | Commercial oil |
|------------------------------------|--------------|----------------|
| Gravity, ° A. P. I.                | 32.4         | 32.3           |
| Sp. gr., 60°/60° F.                | 0.8633       | 0.8639         |
| Lb. gal., 60° F.                   | 7.188        | 7.193          |
| Viscosity, S.U.V.:                 |              |                |
| 70° F.                             | 350          | 349            |
| 100.                               | 154.3        | 154.1          |
| 130.                               | 86.2         | 86.0           |
| 210.                               | 43.5         | 43.4           |
| Viscosity index.                   | 100          | 100            |
| Flash, OC. ° F.                    | 415          | 415            |
| Fire, OC. ° F.                     | 460          | 460            |
| Pour, ° F.                         | 0            | 0              |
| Color, N.P.A.                      | 1.25         | 1.25           |
| Carbon residue, per cent.          | 0.03         | 0.03           |
| Copper strip test, 212° F., 3 hrs. | Passes       | Passes         |
| Neutralization No.                 | 0.04         | 0.04           |
| Iodine No., Mod. Hanus             | 7.14         | 6.9            |

As shown by the above tabulation of properties, the incorporation of this improvement agent in the commercial turbine oil, in the amounts necessary to impart marked rust preventive qualities thereto, did not substantially change any of the above properties thereof. However, the markedly improved rust-preventive qualities of the improved oil so obtained is clearly shown by the results obtained when our improved turbine oil was subjected to the above mentioned standard corrosion test. The data obtained in such test were as follows:

|                                                                                    | Improved oil | Commercial oil |
|------------------------------------------------------------------------------------|--------------|----------------|
| Corrosion test, ASTM D 665-42 T, distilled water 10%, 140° F., 48 hr.—Steel strip: |              |                |
| Appearance.                                                                        | Bright       | Rusted         |
| Area rusted: per cent.                                                             | 0            | 100            |
| Corrosion test, Method 412, Gulf, distilled water, 122° F., 12 days—Steel strip:   |              |                |
| Appearance.                                                                        | Bright       | Rusted         |
| Area rusted: per cent.                                                             | 0            | 100            |

As shown by the above data rusting of steel is entirely prevented with the improved oil.

This improved turbine oil also had other advantageous qualities which render it particularly

useful and advantageous as a lubricant in various types of turbines. When subjected to the various standard tests used in evaluating commercial turbine oils it successfully passed all of them, even the most drastic ones.

For instance, this improved turbine oil is very resistant to emulsification. Further, when emulsions are formed they readily break. This is clearly shown by the data obtained in standard emulsion tests; the results obtained being as follows:

Emulsion test, 180° F.,  
Method 320.13, Gov't:  
Distilled water..... 40-40-0 (4)  
1% salt solution..... 40-40-0 (3)

The above data clearly shows the superior qualities of our improved turbine oils in this respect; these qualities being important in the satisfactory lubrication of turbines.

20 Likewise, our improved turbine oils are resistant to foaming when agitated in the presence of air or gases. Their superiority in this respect is clearly shown by the results obtained when subjected to certain standard foaming tests; the test data obtained being as follows:

Foaming test, Method 413, Gulf:  
550 R. P. M., 15 min.—  
Vol. oil and foam: Vol. oil, 77° F..... 1.00  
After standing 1 hr..... 1.00  
30 900 R. P. M.:  
Vol. oil and foam: Vol. oil, 77° F..... 1.12  
After standing 1 hr..... 1.00

Air bubbling foam test:  
35 Method 435, Gulf—  
Vol. oil and foam: Vol. oil, 77° F..... 1.0  
Vol. oil and foam: Vol. oil, 130° F..... 1.0  
Vol. oil and foam: Vol. oil, 180° F..... 1.0

40 Further, in addition to the above advantageous properties, namely, the marked resistance to foaming and emulsification, and marked anti-corrosion qualities, our improved turbine oils have other superior properties advantageous in lubricating turbines. For instance, they have excellent lubricating qualities as evaluated by the standard "Falex wear test." When so evaluated the test data obtained is as follows:

Falex wear test:  
50 500 lb. gauge load, 15 min.—  
Wear: No. of teeth..... 0  
Gauge load at seizure: Lbs..... 1100

Also, in addition to their excellent lubricating qualities, our improved turbine oils are markedly resistant to oxidation and deterioration. For instance, the improved turbine oils shown in Examples V and VI successfully passed various standard oxidation tests. In one such test, the Sligh oxidation test, the improved turbine oil of 60 Example V had a Sligh oxidation number of 7.

65 In other words, a plurality of advantageous properties can be imparted to turbine oils by incorporating our new improvement agents therein. Likewise, similar improvements can be obtained in other types of lubricants by incorporating our new agents in various oils and oil compositions.

70 For example, our new agents are also useful and advantageous in preparing improved motor oils for lubricating automotive, aviation and Diesel engines. Such improved oils can be readily prepared by incorporating a few per cent of these improvement agents in a suitable mineral lubricating oil; usually 0.3 to 3.0 by weight of the oil. The compounded oils so obtained have im-

proved detergent properties as well as other advantageous properties. In general, such improved motor oils containing minor amounts of our agents have a plurality of advantageous properties. In addition to protecting metals from rust and corrosion, they have superior lubricating properties even under severe operating conditions.

In particular, this invention relates to improved lubricating oils containing a multi-functional improvement agent having antioxidant and other advantageous properties such as high film strength. Moreover, the lubricating oils to which our inhibitor is added are capable of retarding the formation of all forms of gum, resins, carbon, and varnish-like materials which are usually formed on the pistons and rings of internal combustion engines. In addition to the property of being able to inhibit the formation of products capable of corroding sensitive metallic bearings normally found in internal combustion engines or other metals contacted with the oil, all oils containing our improvement agents and minor proportions of water or salt water are inhibited against corrosion tendencies. That is, our improved lubricating compositions comprising a major amount of a petroleum lubricating oil and a minor amount of our new additive compounds have improved detergent, antioxidant and other advantageous properties.

That is, our new improvement agents impart to mineral oil compositions a plurality of advantageous properties which render them particularly advantageous for such purposes. For instance, these improved oil compositions tightly adhere to the metal, forming protective films thereon which are substantially impervious to water and aqueous solutions and which are resistant to removal from the metal even when vigorously agitated with aqueous liquids. That is, our improved oil compositions are markedly resistant to water and aqueous solutions, as well as stable against oxidation.

Accordingly, in the broad practice of this invention a wide range of improved mineral oil compositions can be readily prepared, including excellent protective coating compositions, as well as improved anti-rust lubricants. Thus, broadly, this invention relates to improved mineral oil compositions containing minor amounts of substantially neutral divalent metal salts of N-alkyl, alkylol ortho phthalamidic acids, as a new and advantageous improvement agent; the amount of such improvement agent being sufficient to impart thereto the advantageous properties desired. In general, our improved oil compositions usually contain from 0.03 to 10.0 per cent by weight of such improvement agents dissolved in the mineral oil.

This application is a continuation-in-part of our prior application Serial No. 516,968, filed January 4, 1944, which became U. S. Patent No. 2,378,442 on June 19, 1945, which also relates to improved oil compositions and methods of making the same.

In our said prior application, we have described and claimed improved mineral oil compositions containing a minor amount of oil-soluble calcium phthalyl alkyl amide compounds having the following formula:



wherein R represents an alkyl group containing 8 to 20 carbon atoms. Such oil-soluble compounds can be readily produced from the reaction or inter-action of a polyvalent metal hydroxide, phthalic anhydride and primary alkyl amines, advantageously in situ in mineral oil, as described and illustrated in our prior application. As there shown, the improvement agents so obtained impart a plurality of valuable properties to mineral oils and oil compositions and are advantageous for such purposes.

15 for such purposes.

The oil-soluble calcium phthalyl alkyl amide compounds employed in our prior application are substantially neutral calcium salts of a mono-alkyl amide of phthalic acid, as shown by the above generic formula. They are also designated as calcium N-alkyl amido phthalates, as stated in our prior application. However, as is evident from the above formula, these oil-soluble salts are substantially neutral divalent metal salts of ortho phthalamic acids containing a long chain alkyl group attached to the nitrogen thereof, which carries a reactive hydrogen attached thereto.

25 The oil-soluble salts employed in the present invention are substantially neutral divalent metal salts of ortho-phthalamidic acid containing an alkylol group attached to the nitrogen atom thereof, in addition to the long chain alkyl group attached thereto. Thus, so to speak, our new improvement agents are alkylol derivatives of the improvement agents set forth in our prior application. Indeed, they can be prepared by reacting said neutral calcium phthalyl alkyl amides with propylene oxide and similar alkylene oxides; thereby substituting an alkylol group for the hydrogen attached to the nitrogen atom in the ortho phthalamidic salt shown in our prior application.

40 That is, we have now found that by substituting an alkylol group for the hydrogen attached to the nitrogen atom of the ortho phthalimidic acid salts shown in our prior application, Serial No. 516,968, now U. S. Patent No. 2,378,442, we 45 obtain a new and different class of improvement agents or polyvalent metal salts which in addition to having greater solubility in mineral oils also have other modified properties which render them particularly useful as improvement agents 50 for mineral oils and oil compositions; these improvements being in part due to the presence of the alkylol group in the molecule of our new improvement agents. The present application is broadly directed to improved mineral oil compositions 55 containing these new improvement agents.

What we claim is:

1. An improved mineral oil composition comprising a major amount of a mineral oil and a minor amount of an oil-soluble divalent metal salt of N-alkyl, alkylol ortho phthalamic acid, said metal salt having the following formula



75 wherein M is a divalent metal, R is an alkyl group containing 8 to 22 carbon atoms and R' is hydrogen or an alkyl group, and the amount of said metal salt being sufficient to impart corrosion-

13

inhibiting properties to the improved oil composition.

2. The composition of claim 1 wherein the said mineral oil composition contains from 0.01 to 10.0 per cent by weight of said improvement agent 5 dissolved in the mineral oil.

3. The improved composition of claim 1 wherein the said oil-soluble metal salt is a calcium salt.

4. The improved composition of claim 1 wherein the said oil-soluble metal salt is a substantially 10 neutral calcium salt of N-dodecyl propanol ortho phthalamic acid.

5. An improved mineral oil composition comprising a major amount of a mineral lubricating oil containing dissolved therein from 0.01 to 10.0 per cent by weight of an oil-soluble calcium N- 15

14

alkyl, alkylophthalamic acid salt having the following formula:



wherein R' represents hydrogen or an alkyl group, and n is a number between 6 to 20, said improvement agent being substantially neutral and readily soluble in mineral oils.

HERSCHEL G. SMITH.

TROY L. CANTRELL.

JOHN G. PETERS.

### Certificate of Correction

Patent No. 2,408,103.

September 24, 1946.

HERSCHEL G. SMITH ET AL.

It is hereby certified that errors appear in the printed specification of the above numbered patent requiring correction as follows: Column 3, line 43, before the word "Further" insert the following paragraph—

Processes of making secondary N-propanol N-alkyl amines by reacting equimolecular proportions of propylene oxide and a long chain primary aliphatic amine are claimed in our copending application, Serial No. 640,128, filed January 9, 1946, as a continuation-in-part of the present application. line 63, for the word "is" read *in*; line 67, for "formd" read *formed*; column 4, line 28, for "Txeas" read *Texas*; and that the said Letters Patent should be read with these corrections therein that the same may conform to the record of the case in the Patent Office.

Signed and sealed this 17th day of December, A. D. 1946.

[SEAL]

LESLIE FRAZER,  
*First Assistant Commissioner of Patents.*